# EUROPEAN PATENT SPECIFICATION

(11) **EP 0 416 098 B1**
(45) Date of publication and mention of the grant of the patent: **06.10.1993**
(21) Application number: 88902948.4
(22) Date of filing: 01.04.1988
(51) Int. Cl.: H01F 1/08

(54) **MAGNETICALLY ANISOTROPIC SINTERED MAGNETS**
MAGNETISCH ANISOTROPE SINTERMAGNETE
AIMANTS FRITTES MAGNETIQUEMENT ANISOTROPES

(30) Priority: 29.02.1988 JP 48127/88
(43) Date of publication of application: 13.03.1991
(73) Proprietor: SUMITOMO SPECIAL METALS CO. LTD., Osaka City Osaka (JP)
(72) Inventor: HIROSAWA, Satoshi, Nagaokakyo-shi Kyoto 617 (JP); TOKUHARA, Kohki, Takatsuki-shi Osaka 569 (JP); MAKITA, Ken, Kyoto-shi Kyoto 601-13 (JP); NAGATA, Hiroshi, Mukoh-shi Kyoto 617 (JP)
(74) Representative: Livsey, Gilbert Charlesworth Norris
(86) International application number: JP8800336
(87) International publication number: WO8908318

(56) References cited:
- EP-A- 0 101 552
- EP-A- 0 106 948
- EP-A- 0 126 179
- EP-A- 0 134 304
- EP-A- 0 134 305

## Description

### Technical Field

This invention relates to Fe-B-R based magnetically anisotropic magnets that are not demagnetized when they are mounted on electric motors for vehicles and used in a high temperature environment. The invention provides magnetically an isotopic magnets that do not necessarily require expensive heavy rare earth elements and can keep a high maximum energy product and develop a high coercive force. The invention also provides said magnets at low cost.

### Background Art

The permanent magnet materials are one of very important materials applied to electric and electronic goods and they are used in a very wide area covering various types of home electric appliances, parts for automobiles and communication equipment and peripherals for large scale computers. Recently, with the need for high performance and miniaturization of electric and electronic equipment, high performance permanent magnets are required. Traditionally, the rare earth cobalt magnet is well known to comply with these needs. However, the rare earth cobalt magnet needs a large amount of expensive samarium as the rare earth which is not abundantly contained in the rare earth ore and also needs cobalt at a level of 50-60 weight %.

A ternary compound has previously been proposed by the present applicant which does not necessarily contain rare and expensive samarium or cobalt but does contain light rare earth elements such as neodymium or praseodyraium which elements are abundant in rare earth ore as the main elements and contains iron, boron and the rare earths (R) as the essential elements and thus has excellent magnetic properties with uniaxial magnetic anisotropy by combining the rare earths with iron and boron. Then the applicant has proposed Fe-B-R based magneticall.v anisotropic magnets which develop high permanent magnet properties that far exceed the maximum energy product of the conventional rare earth cobalt magnets. (EPC. Publication No. 83 106 5-13.5).

Permanent magnets have increasingly been exposed to severe environments such as an increase of self-demagnetizing fields due to thinning of magnets, strong demagnetizing fields applied from coils and other magnets, and exposure to high temperature environments due to a tendency to higher speeds and heavier loads for equipment and appliances.

It is well known that the Fe-B-R based magnetically anisotopic sintered magnets show an almost constant temperature coefficient of coercive force (iHc), of about minus 0.6 percent per degree centigrade regardless of some modifications of compositions or manufacturing methods when Nd or Pr are selected as a rare earth element.

Therefore, it is necessary for the magnets to have higher coercive force to be used in the severe environment as mentioned above.

The applicant has further proposed that Fe-B-R based permanent magnets using heavy rare earth elements Dy, Tb as part of (R) comply with this higher coercive force requirement (EP-A-0134305).

But these heavy rare earth elements Dy, Tb are very rare in their ore and also expensive.

As the methods of increasing the coercive force without using these expensive heavy rare earth, the following methods were disclosed in which additive elements M such as V, Cr, Mn, Ni, Mo, Zn and so on are added, or the amount of rare earth Nd, Pr or boron is increased. (EP-A-0101 552).

The method of using the additive elements M has, to be sure, a distinctive effect on the increase in the coercive force by adding M at the level of 1-2 atom %, while more additive M provides little effect on increase in the coercive force when its enhancement is required, and even more of M causes a reduction in the saturation magnetization and forms non-magnetic boride compounds with boron and this brings a rapid decrease in the maximum energy product.

Also, an increase in an amount of rare earth or boron as well as more additive M has been considered to bring a gradual increase of coercive force and rapid decrease in energy product. (EP-A-0101 552, refer to Figs. 3 and 4)

In view of these situations at present, the object or this invention is to provide the Fe-B-R based magnetically anisotropic sintered magnets which do not necessarily need expensive heavy rare earth elements and do not cause a rapid decrease in maximum energy product due to increase in coercive force, retaining more than 20MGOe (1 G = 10-⁴ T, 1 Oe = 103/4-ff Am-') and having high coercive force more than 15kOe (1 Oe = 10³/4_{7T} Am-') .

### Disclosure of Invention

In this invention, compositions of Fe-B-R based magnetically anisotropic sintered magnets were considered to improve the coercive force by increasing an amount of B, and as a result of these considerations, it was found that an amount as small as impurity level contained in industrial raw materials give rise to an increase in coercive force and said sintered magnets have a very large coercive force without reducing the maximum energy product are obtained by controlling the amount of these elements represented below.

That is, the fact described below was found that , by including in the material a small amount of solutes such as Al, Si, Cu, Cr, Ni, and Mn effective for enhancing the coercive force and excluding from the material harmful impurities such as P, S, and Sb, and then powdering this material by usual melting, casting, crushing, or direct reduction method and subjecting this powder to orientation in a magnetic field, compacting, sintering and optionally subjecting the material to heat treatment, Fe-B-R based sintered magnets were obtained that have a maximum energy product more than 20MGOe (1 G = 10-⁴ T, 1 Oe = 10³/4π Am-') and a coercive force more than 15kOe (1 Oe = 10³/4π Am⁻¹) .

The present invention provides a magnetically anisotropic sintered magnet which comprises, by atomic percent:
(i) 14.0-18.0% of (R)
   wherein (R) is the total of:
   0-18.0% Nd
   0-18.0% Pr
   0-2.5% Dy
   0-2.5% Tb,
   provided that the total of Dy + Tb does not exceed 2.5%;
(ii) 9.0-18.0% of boron
(iii) 0.5-5.0% of "A"
   wherein "A" is the total of:
   0.20-2.0% AI
   0.01-0.5% Si
   0.03-0.6% Cu,
   and at least one of:
   0.02-3.0% Cr
   0.05-1.0% Mn
   0.02-1.0% Ni;
(iv) 0-10% cobalt;
(v) and the balance is iron.

The present invention also provides such a magnet which additionally comprises:
(a) one or more of V, Mo, Nb, W, in an amount of less than 2.0%; and
(b) one or more of Zn, Ti, Zr, Hf, Ta, Ge, Sn, Bi, Ca, Mg in an amount of less than 1.0%;
   wherein the total of (a) + (b) is less than 2.0%.

### Detailed Description of Preferred Embodiments of the Invention

In this invention, the rare earths (R) at least comprise one of Nd and Pr, and one of them is usually used to satisfy requirement but a mixture of them may be used to comply with circumstance of material procurement.

If the content of (R) is less than 14 at%, a large coercive force more than 15kOe (1 Oe = 103/4π Am-') , that is the characteristic of this invention, is not obtained and if the content exceeds 18 at %, the residual magnetic flux density (Br) decreases and a value more than (BH)max 20MGOe (1 G = 10-⁴ T, 1 Oe = 103/4π Am-') is not obtained, therefore the content is maintained within the range of 14 at%-18 at%.

The content of (R) within the range of 15 at%-17 at% permits the magnets to obtain coercive forces more than 18kOe (1 Oe = 103/4π Am-') without decreasing (BH)max, and therefore this range is preferable.

In this invention, more than 9 at% of B is required to obtain the maximum energy product above 20MGOe (1 G = 10-⁴ T, 1 Oe = 103/4π Am⁻¹) and the coercive force above 15kOe (1 Oe = 103/4π Am⁻¹) , however more than 18 at% B decreases the residual magnetic flux density, therefore the amount of B should be limited within the range of 9 at%-18 at%.

Further, a content of B within the range of 10 at%-17 at% permits the magnets to obtain coercive forces of more than 18kOe (1 Oe = 103/4π Am-') without addition of heavy rare earths elements. This range is therefore especially preferable.

It is known that the Fe-B-R based sintered magnets have a tetragonal crystal structure and compounds indicated by a formula R₂Fe₄B determine magnetic properties. The compounds exist in a sintered body as crystal grains having mean particle diameters of 1-20µm. Both an (R)-rich phase which is almost occupied by rare earth and a B-rich phase indicated by R_{1.1} Fe4 B4 play important roles in the mechanism of coercive force.

It is supposed that the reason why a very small amount of additive elements "A" characterized in this invention has great effect on coercive force enhancement is because the additives effectively act on circumferences of the tetragonal crystal particles, that support the magnetic performance of the sintered magnet within the range of several atomic layers.

In this invention, a very small amount of the essential elements Al, Si and Cu among the additives develops distinctive enhancement of coercive force. In order to obtain such an effect, at least an amount of AI of more than 0.2 at% content, Si of more than 0.01 at% content, and Cu of more than 0.03 at% content is required.

Further, for the purpose of obtaining a maximum energy product of more than 20MGOe (1 G = 10-⁴ T, 1 Oe = 103/4-ff Am-') and a coercive force of more than 15kOe (1 Oe = 103/4-ff Am-'), an amount of AI of less than 2.0 at% content and Si of less than 0.5 at% content is required. If the Cu content exceeds 0.6 at%, the coercive force on the contrary decreases. Thus the content of Cu should be limited to less than 0.6 at%.

In addition, by including a very small amount of at least one of Cr, Mn and Ni, namely more than 0.02 at% Cr, more than 0.05 at% Mn and more than 0.02 at% Ni has a good effect on the coercive force enhancement.

However, a relatively large amount of Cr, Mn and Ni causes degradation of magnetic properties of elevated temperatures through a considerable decrease in Curie temperature or causes on the contrary coercive force decrease. Thus amounts of less than 3.0 at% Cr and less than 1.0 at% Mn are required. If the Ni content exceeds 1.0 at%, coercive force decreases. Thus the content of Ni is required to be less than 1.0 at%.

When a total amount of adding of the additive elements "A", namely, Al, Si, Cu, Cr, Mn and Ni is less than 0.5 at%, this has no good effect on coercive force enhancement. A total amount of "A" exceeding 5.0 at% causes the decrease of the maximum energy product. Thus the range of 0.5 at%-5.0 at% "A" should be observed.

Further, in this invention,at least one of V, Mo, Nb and W and at least one of Zn, Ti, Zr, Hf, Ta, Ge, Sn, Bi, Ca, Mg and Ga may be added to enhance coercive force and even only as small an amount as 0.1 at% can enhance coercive force.

However, if the magnet contains at least one of V, Mo, Nb an W each having a content more than 2.0 at%, or at least one of Zn, Ti, Zr, Hf, Ta, Ge, Sn, Bi, Ca, Mg and Ga each having content more than 1.0 at%, and further if the total amount of these selected elements exceeds 2.0 at% content, this causes a decrease in the maximum energy product and such amounts are not preferable.

Co raises the Curie temperature of the Fe-B-R based permanent magnets and improves the temperature characteristic of the residual magnetic flux density and anti-corrosive properties. To obtain these effects, an amount of Co of more than 0.1 at% of the magnet content is required. However a relatively large amount yields RCo intermetallic compounds that decrease coercive force. Thus amounts of less than 10 at% are preferable.

When at least one of Mn, Cr and Ni are added so that a total content is more than 0.5 at%, this produces an advantage that oxidation of the fine powder material during processing can be reduced.

When Cr is added to produce a content more than 1.0 at%, the anti-corrosive properties of the alloy powder and the finished products can be remarkably improved.

When the permanent magnets of this invention are manufactured, sometimes they contain 0₂ or C. That is, the magnets contain them at each stage of processing such as raw material, melting, crushing, sintering and heat treatment. A content less than 8000 ppm does not damage the effect of this invention but a content less the 6000 ppm is preferable.

Sometimes C may be contained in materials or it is added as binder or lubricant of improve moldability of the compact after pressing. A content less than 3000 ppm during sintering does not damage the effect of this invention but a content less than 1500 ppm is preferable.

This invention allows the magnets to obtain large coercive forces not necessarily requiring the heavy rare earth as (R) and permits further improvement of coercive force enhancement by replacing said Nd, Pr with a small amount of Dy, Tb if necessary.

If the amount of replacement by Dy, Tb is more than 0.05 at%. the effect of the coercive force enhancement is obtained and even a small amount of additives yields the equivalent or greater effect than that obtained from said conventional positive addition of Dy, Tb. Therefore the upper limit of this positive addition of Dy, Tb should be limited to 2.5 at% of the magnet.

A concentration range large than 0.5 at% is the preferable as the concentration of Dy and Tb, because it provides iHc larger than 20kOe (1 Oe = 103/4π Am-¹) maintaining 20MGOe (1 G = 10-⁴ T, 1 Oe = 103/4π Am⁻¹) .

### Method of making

Alloy powder having Fe-B-R compositions is first obtained as starting material.

After the material is alloy-melted in an usual manner, an alloy ingot is obtained from, for example, casting cooled in the condition that does not cause an amorphous state. This alloy ingot is then crushed, classified and mixed to produce alloy powder, or alloy powder obtained from rare earth oxides by reduction by Ca or Mg may be used (direct reduction method).

Mean particle size should be within the range of 0.5-10µm.

Mean particle size of 1.0-5µm is the most preferable to obtain excellent magnetic properties.

Crushing may be implemented both by wet crushing that is performed in a solvent or by dry crushing that is performed in a gas atmosphere such as N₂. The jet mill used in dry crushing yields uniform powder particle size and this is recommended to obtain a higher coercive force.

Then the alloy powder is compacted and this compacting may be carried out in the same manner as in conventional powder metallurgy. Pressurized molding is preferable and alloy powder, for example, is pressed and compacted at a pressure of 0.5-3.0 ton/cm² in a magnetic field the intensity of which is more than 5kOe (1 Oe = 103/4-ff Am-') to acquire anisotropy.

Sintering of the compacted body is carried out in a deoxidizing or non-oxidizing atmosphere at a predetermined temperature within the range of 900-1200 ° C. This is recommendable.

For example, the compacted body is sintered at a temperature within the range of 900-1200 ° C for 0.5-4 hours in a vacuum less than 10-² Torr, or in an inert gas or a deoxidizing gas atmosphere with 1-76 Torr and gas purity more than 99 %.

The sintering is performed adjusting the conditions of temperature and time in order to acquire a predetermined crystal particle diameter and density in the sintered body.

The density of the sintered body is preferably more than 95 % of the theoretical density (ratio), for example, a density more than 7.2 g/cm³ is acquired at a sintering temperature within the range of 1040-1160°C, and this corresponds to more than 95 17,₀ of the theoretical density. Furthermore, more than 99 % theoretical density ratio is obtained within the range of 1060-1100 ° C and this is especially preferable.

Heat treatment of the sintered body at a temperature withlin the range of 400-900 ° C for 0.1-10 hours is effective to further improve coercive force. In these heat treatment temperature conditions, the sintered body may be maintained at a required constant temperature or may be gradually cooled or subjected to multi-stage heat-treating within a predetermined temperature range.

It is preferable that the heat treatment is implemented in a vacuum, or in an inert gas or deoxidizing gas atmosphere.

The heat treatment of the Fe-B-R based sintered magnets is effectively performed under the condition that after sintering, the body is initially held at a temperature within the range of 650-900 ° C for 5 minutes-10 hours. Thereafter, the body is subjected to multi-stage heat treatment, two or more stages of which are carried out at a temperature lower than that of one-stage aging.

### Brief Description of Drawings

Fig. 1 shows the relationship between boron concentration an coercive force iHc.

Fig. 2 shows the relationship between boron concentration and maximum energy product (BH)max.

### EXAMPLES

### Example 1

Ingots having 15NdxB(100-x)Fe in at% (x=4 - 25) compositions were manufactured by melting, using: fineness 97 wt% Nd (the remainder is almost rare earth elements such as Pr), electrolytic iron (Si, Mn, Cu, AI and Cr each having wt% less than 0.005 wt%)

and as B
(1) commercially available ferroboron (equivalent to JIS G2318 FBL1; 19.4 wt% B, 3.2 wt% Al, 0.74 wt% Si, 003 wt% C, the remainder being composed of other impurities and Fe.)
(2) commercially available high fineness boron of fineness 95% or larger containing little impurities.

Further, as (3) those ingot embodiments of this invention containing 0.4 at% Al, 0.3 at% Si, 0.15 at% Cu, 0.08 at% Mn, 0.5 at% Cr and 0.3 at% Ni were similarly manufactured by substituting for Fe in material (2).

These ingots were roughly crushed by a jaw crusher and finely pulvelized in a N² gas atmosphere by a jet mill and fine particle powder having mean particle size of 3.3-3.6µm was finally obtained.

This material powder was compacted with pressure of 1.5 ton/cm² in a magnetic field applied perpendicular to the press direction, the intensity of which was 10k0e (1 Oe = 103/4-ff Am⁻¹) . The compacted body thus obtained was subjected to sintering at a temperature within the range of 1040-1100°C and the sintered body having the theoretical density ratio more than 96 % was obtained.

Further, these sintered bodies were heat-treated by 25 ° C steps for 2 hours within the range of 900-400 _{°} C. The specimens having the best magnetic properties were picked up and their magnetic properties were measured at room temperature (22 ° C) and compared to one another on the basis of property variations vs boron amounts added.

Variations of coercive force are shown in Fig. 1 and variations of the maximum energy product are shown in Fig. 2. The curves of the maximum energy product derived from each material (1), (2) and (3) show almost no difference, however the curve (1) of the coercive force derived from the material (1), namely, the commercially available ferroboron whose impurities are not controlled shows no effect of increasing coercive force at the point of about 10 at% boron concentration and thereafter.

Further, the curves show if the high fineness boron is used that does not contain the very small amount elements used in this invention, a considerable amount of boron must be used as compared with the embodiments of this invention to acquire a predetermined coercive force.

On the contrary, the sintered magnet according to the invention has an energy product more than 20MGOe (1 G = 10-⁴ T, 1 Oe = 103/4π Am-') and keeping this condition, a large coercive force is obtained as shown in Figs. 1 and 2.

### Example 2

Similarly to Example 1, ingots having 16Nd9B remainder Fe based compositions in at% were made in which the following additives were substituted for Fe: 0.5 at % Al, 0.18 at % Si, 0.12 at % Cu, 0.3 at % Mn, 0.5 at % Cr and 0.5 at % Ni (total 2.1 at %). The effect of the elements on the magnetic properties was studied. Measurements of the coercive force are shown in Table 1.

As can be seen from Table 1, the effect of Al, Si and Cu is remarkable and if any one of these elements is absent, the coercive force decreases.

Concerning Mn, Cr and Ni, existence of any one of these can keep the coercive force from decreasing. Lack of these elements decrease the coercive force.

### Example 3

Similarly to Example 1, the magnets having 0.5 at% Al, 0.15 at% Cu, 0.18 at% Mn, 0.3 at% Si and 0.5 at% Cr (= "A", total 1.63 at%) of very small amount elements were manufactured. Measurements of the magnetic properties are shown in Table 2.

### Industrial Applicability

The magnets according to this invention are pressed to a direction perpendicular to a magnetic field, sintered and subjected to heat treatment. By these processes the magnets can have a maximum energy product more than 20MGOe (1 G = 10-⁴ T, 1 Oe = 103/4π Am⁻¹) and a coercive force more than 15kOe (1 Oe = 103/4-ff Am-') and develop stable magnetic properties than 150 _{°} C. Sintered magnets obtained by pressing in a magnetic field applied parallel to the press direction followed by sintering and optional heat treatment have a smaller energy product than the above said magnets, but are good enough to be used practically.

The sintered magnets according to the invention are characterized in that they have a high content of B and very small amounts additive elements. Even though the B content is increased more than several at%, the weight of the magnet increases little, and the added amount of the additive elements "A" is very small, therefore high coercive force magnets can be obtained without changing the conventional manufacturing method.

In addition, mechanical strength such as flexural strength does not vary regardless of the increase in boron concentration and high mechanical strength can be obtained that is the characteristic of the Fe-B-R based magnets.

Further, the magnets according to the invention do not have worsening of the bending characteristic of the demagnetizing curve, but have an excellent bending characteristic.

Still further, this invention is characterized in that the magnets do not necessarily need the heavy rare earth elements and has an advantage that if a large coercive force, for instance, larger than 20kOe (1 Oe = 10³/4π Am⁻¹) is required, the addition of a very small amount of Dy and Tb may satisfy the requirement.

As can be seen from the embodiments, the improvement of the coercive force can not be obtained from using only materials already containing AI or Si and commercially available ferroboron or boron containing a relatively large amount of impurities. The effect of this invention is not acquired until the materials are controlled to contain predetermined contents of additives according to the invention.

## Claims

1. A magnetically anisotropic sintered magnet which comprises, by atomic percent:
(i) 14.0-18.0% of (R)
wherein (R) is the total of:
0-18.0% Nd
0-18.0% Pr
0-2.5% Dy
0-2.5% Tb,
provided that the total of Dy + Tb does not exceed 2.5%;
(ii) 9.0-18.0% of boron
(iii) 0.5-5.0% of "A"
wherein "A" is the total of:
0.20-2.0% AI
0.01-0.5% Si
0.03-0.6% Cu,
and at least one of:
0.02-3.0% Cr
0.05-1.0% Mn
0.02-1.0% Ni;
(iv) 0-10% cobalt;
(v) and the balance is iron.

2. A magnet as claimed in claim 1, which additionally comprises:
(a) one or more of V, Mo, Nb, W, in an amount of less than 2.0%; and
(b) one or more of Zn, Ti, Zr, Hf, Ta, Ge, Sn, Bi, Ca, Mg in an amount of less than 1.0%; wherein the total of (a) + (b) is less than 2.0%.

## Patentansprüche

1. Ein magnetisch anisotroper Sintermagnet, der in Atom-% enthält:
(i) 14,0-18,0% an (R),
wobei (R) die Gesamtheit von:
0-18,0% Nd
0-18,0% Pr
0-2,5% Dy
0-2,5% Tb ist,
vorausgesetzt das die Gesamtheit von Dy + Tb 2,5% nicht überschreitet;
(ii) 9,0-18,0% Bor
(iii) 0,5-5,0% an "A",
wobei "A" die Gesamtheit von:
0,20-2,0% AI
0,01-0,5% Si
0,03-0,6% Cu ist sowie mindestens einer der Anteile von
0,02-3,0% Cr
0,05-1,0% Mn
0,02-1,0% Ni;
(iv) 0-10% Kobalt;
(v) der Ausgleich ist Eisen.

2. Ein Magnet nach Anspruch 1 der zusätzlich enthält:
(a) Eine oder mehrere der Komponenten V, Mo, Nb, W in einem Anteil von weniger als 2,0% und
(b) eine oder mehrere Komponenten Zn, Ti, Zr, Hf, Ta, Ge, Sn, Bi, Ca, Mg in einem Anteil von weniger als 1,0%, wobei die Gesamtheit von (a) + (b) weniger als 2,0% beträgt.

## Revendications

1. Un aimant fritté magnétiquement anisotrope qui comprend, en pourcentage atomique :
(i) 14,0-18,0% de (R)
en désignant par (R) le total de :
0-18,0% de Nd
0-18,0% de Pr
0-2,5% de Dy
0-2,5% de Tb,
le total de Dy + Tb ne dépassant pas 2,5%.
(ii) 9,0-18,0% de bore
(iii) 0,5-5,0% de "A"
en désignant par "A" le total de :
0,20-2,0% de AI
0,01-0,5% de Si
0,03-0,6% de Cu,
et l'un au moins des éléments suivants:
0,02-3% de Cr
0,05-1,0% de Mn
0,02-1,0% de Ni;
(iv) 0-10% de cobalt;
(v) et le complément en fer.

2. Un aimant selon la revendication 1, qui comprend en outre :
(a) un ou plusieurs des éléments : V, Mo, Nb, W, en une proportion inférieure à 2,0%; et
(b) un ou plusieurs des éléments Zn, Ti, Zr, Hf, Ta, Ge,
Sn, Bi, Ca, Mg en une proportion inférieure à 1,0%; dans lequel le total (a) + (b) est inférieur à 2,0%.
